

Patented Aug. 16, 1927.

1,639,395

# UNITED STATES PATENT OFFICE.

CHARLES R. BRAGDON, OF CINCINNATI, OHIO, ASSIGNOR TO THE AULT & WIBORG COMPANY, OF CINCINNATI, OHIO, A CORPORATION OF OHIO.

## ADHESIVE LACQUER OR VARNISH COMPOSITION.

No Drawing.

Application filed January 16, 1926. Serial No. 81,771.

This invention relates to a novel adhesive lacquer or varnish composition and consists of the matters hereinafter described and more particularly pointed out in the appended claims.

The novel lacquer or varnish is of especial value for use on the inside faces of caps or so-called crown corks adapted to be applied and clamped to the tops of bottles 10 and jars for sealing them. Within each of said caps is contained a cork or other resilient sealing disc which directly engages the top lip of the bottle or jar in such manner as to provide an hermetical seal to prevent 15 contamination of the contents. Such discs are preferably cemented to the inside faces of the caps by an adhesive compound, and the lacquer or varnish described herein is designed to act as such adhesive.

Crowns or caps of the kind are generally stamped and formed from thin metal sheets,—a large number of such caps being cut from a single sheet. The disc of cork or other resilient material which is to provide 20 the seal, is then cemented by some adhesive compound within the cap. Several kinds of cementing compound have been used, among them being one based on egg albumen and others consisting of resins dissolved in alcohol. Most of these compounds 25 are applied in liquid form by means of a dropper to the finished caps individually when the sealing disc is inserted into the cap.

The application of such adhesive compounds applied in this manner is tedious and time-consuming and adds considerably to the expense of manufacture of the crowns or caps. In addition, adhesive compounds 30 applied in this way are not very efficient in maintaining the adhesion of the disc to the cap.

The object of my invention is to provide an improved adhesive lacquer or varnish, 45 which may be applied in a single operation by a coating machine to one side of the metal sheet from which the crowns or caps are to be stamped, so that the adhesive is already on the inside of the caps when they 50 are formed. The step of separately applying adhesive cement to each cap or crown is thereby eliminated and the cost of manufacture of the crowns or caps greatly reduced. In addition, the novel lacquer or

varnish provides a more efficient and permanent adhesion of the disc to the cap.

My improved lacquer or varnish, after it is applied to the flat metal sheet by the coating machine, is dried, preferably by baking the sheet in an oven at a temperature of 60 from 180° to 250° F., wherein it is allowed to remain from twenty minutes to half an hour. When the sheets are removed from the oven, they may then be piled one upon the other without danger of the sheets sticking together.

After the sheets have been passed through the die stamping machines, the formed crowns or caps are then passed through assembling machines, in which each cap has 70 inserted into it a cork or other sealing disc. The caps or crowns are next passed over small gas flames or other source of heat for a few seconds to soften the lacquer or varnish. They are then subjected to pressure 75 between plungers which hold the sealing discs against the inner surfaces of the crowns or caps until they are cooled. This finishes the operations,—the sealing discs being then firmly cemented to the crowns or 80 caps.

With the method of handling the sheets from which the caps are made, as above outlined, it is evident that two apparently opposed requirements are to be met with a 85 varnish adhesive of the kind. The varnish must not be so "tacky" or sticky after application, baking and cooling, that it will cause the metal sheets to stick together when piled one upon the other. Upon the other 90 hand, it must have sufficient adhesive quality to efficiently and permanently hold the sealing disc to the cap without danger of the disc becoming detached from the cap. These apparently opposed characteristics 95 are to be found in the improved lacquer or varnish composition herein described.

In addition said composition possesses the required properties for satisfactory application by means of a coating machine and is free from any ingredients that might contaminate the contents of the bottles or jars to which the crowns or caps are applied, in case the said contents should penetrate the sealing disc and come in contact with the lacquer or varnish.

My improved lacquer or varnish composition consists of a mixture of—(1) a com-

bination of varnish resins, hard copal resin or gum and rosin or colophony; (2) asphaltum or pitch; (3) a combination of drying and semi-drying oils; (4) a small amount 5 of calcium hydrate; (5) and a small amount of resinate of manganese. The mixture of these elements constitutes the body of the composition,—that is to say, the part which remains on the metal sheet after the sheet 10 has been baked. This mixture is made into liquid form capable of application by a coating machine by the addition of (6) mineral spirits such as naphtha or turpentine substitute, with which it is thoroughly 15 intermixed.

In preparing the lacquer or varnish composition, I prefer to use the ingredients in about the following proportions:—(1) 427 lbs. of varnish resins consisting of 300 lbs. 20 of wood rosin and 127 lbs. of Congo copal gum; (2) 17½ lbs. of gilsonite asphaltum; (3) 323 lbs. of drying and semi-drying oils, comprised of 237 lbs. of heavy-bodied prepared linseed oil, and 76 lbs. of prepared 25 tung oil, 5 lbs. of Menhaden oil and 5 lbs. of soya bean oil; (4) 3 lbs. of calcium hydrate; and (5) ¾ lb. of resinate of manganese. This is mixed with (6) 593 lbs. of 30 mineral spirits (naphtha and turpentine substitute.)

Another good example of ingredients for the composition is the following:—

(1) 405 lbs. of varnish resins consisting of 275 lbs. of wood rosin and 130 lbs. of 35 Congo copal gum; (2) 35 lbs. of gilsonite asphaltum; (3) 320 lbs. of drying and semi-drying oils, comprised of 220 lbs. of heavy-bodied linseed oil, 80 lbs. of prepared tung oil, 10 lbs. of Menhaden oil; 10 lbs. of soya 40 bean oil; (4) 2 lbs. calcium hydrate; and (5) ¾ lb. of resinate of manganese. With this is mixed (6) 600 lbs. of mineral spirits (naphtha and turpentine substitute).

The above two examples illustrate the 45 manner in which the proportions of the ingredients of the composition may be varied. The gilsonite asphaltum or pitch will vary according to the color desired in the lacquer or varnish. These may be referred to as 50 bitumen or binuminous material, a term intended to include either pitch or gilsonite, when used in the claims. The rosin may be derived from either scraping of the pine tree so-called gum rosin or from extraction 55 from the wood itself or wood rosin.

Good results may be obtained wherein the ingredients are varied within the following limitations,—that is to say (1) from 250 to 60 450 lbs. of varnish resins of which 120 to 130 lbs. is hard copal resin, the balance being wood rosin; (2) from 15 to 35 lbs. of gilsonite asphaltum (asphaltum or pitch); (3) from 300 to 350 lbs. of drying 65 and semi-drying oils of which 220 to 240 lbs. may be heavy-bodied prepared linseed

oil, 75 to 80 lbs. of prepared tung oil, and the balance Menhaden and soya bean oils, in substantially like amounts; (4) from 2 to 3 lbs. of calcium hydrate; and (5) from ¾ to 1 lb. of resinate of manganese. The 70 amount of (6) mineral spirits to be mixed with this varies from 550 to 600 lbs.

I claim as my invention:—

1. A lacquer or varnish composition which is non-adhesive at ordinary temperatures 75 after baking, but which will become strongly adhesive when subsequently heated, which includes a mixture of varnish resins, consisting of copal resin and rosin; drying and semi-drying oils; calcium hydrate; resinate of manganese; and a bituminous coloring material.

2. A lacquer or varnish composition which is non-adhesive at ordinary temperatures after baking, but which will become strongly 80 adhesive when subsequently heated, which includes a mixture of varnish resins, consisting of copal resin and rosin; drying and semi-drying oils; calcium hydrate; and resinate of manganese. 85

3. A lacquer or varnish composition which is non-adhesive at ordinary temperatures after baking, but which will become strongly adhesive when subsequently heated, which includes a mixture of varnish resins, consisting of copal resin and rosin; drying and semi-drying oils; calcium hydrate; resinate of manganese; and a bituminous coloring material;—the mixture being reduced to 90 liquid form by the addition of mineral 95 spirits.

4. A lacquer or varnish composition which is non-adhesive at ordinary temperatures after baking, but which will become strongly adhesive when subsequently heated, which includes a mixture of varnish resins, consisting of copal resin and rosin; drying and semi-drying oils; calcium hydrate; and a resinate of manganese;—the mixture being 100 reduced to liquid form by the addition of mineral 105 spirits. 110

5. A lacquer or varnish composition which is non-adhesive at ordinary temperatures after baking, but which will become strongly adhesive when subsequently heated, which includes a mixture of varnish resins, consisting of copal resin and rosin; drying and semi-drying oils; calcium hydrate; resinate of manganese; and a bituminous coloring material,—substantially in the proportions 115 as described, the mixture being reduced to liquid form by the addition of mineral 120 spirits.

6. A varnish or lacquer composition including a mixture of from 250 to 450 lbs. of varnish resins of which 120 to 130 lbs. is hard copal resin, the balance being wood 125 rosin; from 15 to 35 lbs. of gilsonite asphaltum; from 300 to 350 lbs. of drying and semi-drying oils of which 220 to 240 lbs. are 130

heavy-bodied prepared linseed oil, 75 to 80 lbs. are prepared tung oil, and the balance, Menhaden and soya bean oils, in substantially like amounts; from 2 to 3 lbs. of calcium hydrate; and from  $\frac{3}{4}$  to 1 lb. of resinate of manganese.

7. A varnish or lacquer composition including a mixture of from 250 to 450 lbs. of varnish resins of which 120 to 130 lbs. are 10 hard copal resin, the balance being wood rosin; from 15 to 35 lbs. of gilsonite asphaltum; from 300 to 350 lbs. of drying and semi-drying oils of which 220 to 240 lbs. are heavy-bodied prepared linseed oil, 75 to 80 15 lbs. are prepared tung oil and the balance, Menhaden and soya bean oils, in substantially like amounts; from 2 to 3 lbs. of calcium hydrate; and from  $\frac{3}{4}$  to 1 lb. of resinate of manganese,—the mixture being reduced to liquid form by the addition of 550 20 to 600 lbs. of mineral spirits.

8. A varnish or lacquer composition including a mixture of 427 lbs. of varnish resins consisting of 300 lbs. of wood rosin 25 and 127 lbs. of Congo copal gum; 17½ lbs.

of gilsonite asphaltum; 323 lbs. of drying and semi-drying oils, comprised of 237 lbs. of heavy-bodied prepared linseed oil, 76 lbs. of prepared tung oil, 5 lbs. of Menhaden oil and 5 lbs. of soya bean oil; 3 lbs. of calcium 30 hydrate; and  $\frac{3}{4}$  lb. of resinate of manganese, —the mixture being reduced to liquid form by the addition of mineral spirits.

9. A varnish or lacquer composition including a mixture of from 250 to 450 lbs. of varnish resins of which 120 to 130 lbs. is 35 hard copal resin, the balance being wood rosin; from 300 to 350 lbs. of drying and semi-drying oils of which 220 to 240 lbs. are heavy-bodied prepared linseed oil; 75 to 40 80 lbs. are prepared tung oil, and the balance, Menhaden and soya bean oils, in substantially like amounts; from 2 to 3 lbs. of calcium hydrate; and from  $\frac{3}{4}$  to 1 lb. of 45 resinate of manganese.

In testimony that I claim the foregoing as my invention, I affix my signature this 14th day of January, A. D. 1926.

CHARLES R. BRAGDON.